

April 7, 1931.

W. WILDERMUTH

1,799,203

METHOD OF OPERATING A SHEET GLASS SUPPORTING MEANS

Filed June 29, 1929



Willian Wildermuth

By *Frank Fraser*  
Attorney

## UNITED STATES PATENT OFFICE

WILLIAM WILDERMUTH, OF LANCASTER, OHIO, ASSIGNOR TO LIBBEY-OWENS-FORD  
GLASS COMPANY, OF TOLEDO, OHIO, A CORPORATION OF OHIO

## METHOD OF OPERATING A SHEET-GLASS-SUPPORTING MEANS

Application filed June 29, 1929. Serial No. 374,764.

The present invention relates to an improved method and apparatus for forming sheet or plate glass.

The invention has utility when incorporated in apparatus for the production of sheet or plate glass by a continuous or substantially continuous drawing or rolling operation or in any other apparatus wherein it is desired to support a glass sheet while in a semi-plastic condition.

An important object of the invention is in the provision of movable means for supporting the glass sheet while in a semi-plastic condition and operable in such a manner as to facilitate the flattening of the sheet and minimize the danger of the sheet being marked or marred by said supporting means.

Another object of the invention is to provide a movable table for supporting a moving sheet of glass thereupon while in a semi-plastic condition, said table traveling in the same direction as the sheet but preferably at a relatively slower rate of speed.

Other objects and advantages of the invention will become more apparent during the course of the following description when taken in connection with the accompanying drawings.

In the drawings forming a part of this application and wherein like numerals are employed to designate like parts throughout the same,

Fig. 1 is a fragmentary vertical sectional view through apparatus provided by the present invention.

Fig. 2 is a top plan view of a portion of one type of glass supporting table, and

Fig. 3 is a similar view showing a somewhat modified type of table.

While the invention has been herein disclosed as used in connection with sheet rolling apparatus, it is to be understood that it is not restricted to such use but, on the other hand, may also be incorporated in sheet drawing apparatus of the type disclosed in the Colburn Patent 1,248,809 or in any other apparatus wherein it is desired to support a moving sheet while in a semi-plastic condition.

Referring to Fig. 1 of the drawings, the

numeral 5 designates a working receptacle adapted to contain a mass of molten glass 6 which may be supplied thereto either continuously or substantially continuously from any suitable type of furnace, not shown. 55 The working receptacle 5 is supported on stools 7 contained in a chamber 8, the temperature of which may be controlled by means of burners or the like 9 operating through ports 10. 60

Positioned transversely of the pot 5 is a pair of rolls 11 and 12 respectively, these rolls being so positioned that the lower periphery of said rolls may be arranged within the pot in a manner that they just contact with the surface of the molten glass 6. The rolls are adapted to be positively driven and mounted with respect to one another to create a sheet forming pass therebetween. A heavy meniscus or source of supply 13 furnishes 70 sufficient glass to the sheet forming pass between the rolls 11 and 12 to allow an actual rolling in contradistinction to a drawing operation such as in the use of the regular Colburn machine disclosed in the patent 75 noted above. As shown, after the sheet 14 has been formed, it is moved vertically from the sheet forming pass and is adapted to be deflected over a third roll 15. This roll is positioned in a relatively higher horizontal 80 plane than the roll 16 and the series of rolls 17. The roll 16 is mounted in the same horizontal plane as the rolls 17 and is of sufficient size so that it can be used as a deflecting roll if desired. That is, the sheet, instead of being trained about the roll 15, can be deflected 85 over the forming roll 11 and passed directly to the roll 16.

Adjacent the series of rolls 17 and adapted to receive the glass sheet 14 therefrom is a sheet supporting and flattening table designated in its entirety by the numeral 18 and consisting preferably of a plurality of links pivotally associated with one another in endless belt formation. The adjacent links may be spaced from one another as illustrated in Fig. 2 to provide an open work construction or the said links may abut one another as in Fig. 3, to present a table having a substantially solid unbroken surface. The endless 100

table 18 is trained about sprockets or drums 19 and 20 either one of which or both may be positively driven, while the upper horizontal run of the table is moved over stationary 5 table rails 21 or the like so that a substantially flat sheet supporting surface will be provided for the sheet during its flattening period.

The table 18 is preferably arranged in the 10 temperature controlled compartment 22 and, as shown, heating means 23 are used to control the temperature of the compartment in which the table is contained. The flames from the burners 23 are directed through 15 openings 24 in the bottom of compartment 22 and above either one or both of these openings may be placed a substantially horizontal perforated slab 25 supported on blocks 26. The perforated slab breaks up or diffuses 20 the flame issuing from the burner and permits a more uniform application of heat to the compartment 22 and flattening table 18. An annealing leer 27 is arranged adjacent the flattening table and may include a series of 25 positively driven rolls 28 upon which the sheet may be supported and conveyed therethrough. The annealing of the glass sheet will be readily understood by those versed in the art.

30 The above generally sets forth the formation of the sheet and the manner in which it is handled until it reaches the annealing leer. The present invention, however, particularly concerns the manner in which the 35 flattening table 18 is adapted to be operated so as to give a better flattening of the sheet and improve the quality thereof. Heretofore, the table 18 has been driven at substantially the same speed as the travel of the 40 sheet and, in fact, has been driven at such a speed as to maintain the sheet under a slight tension without, however, causing any reduction in the thickness thereof. When so operated, the glass sheet would lie upon the 45 table for a considerable length of time sufficient to allow the sheet, because of its plasticity, to settle upon the table and be marked or marred by the links thereof. In accordance with the present invention, the flattening table 18 is adapted to be moved in the 50 same direction as the sheet but at a variable and preferably slower speed. When driving the table at a speed relatively slower than the speed of travel of the sheet, no portion 55 of the sheet will lie over any one point of the table continuously during the time it is traveling thereon. Since the point of contact between the glass sheet and table is constantly changing, a better and more efficient flattening of the sheet will be achieved. Also, this 60 will eliminate the checkered appearance sometimes taken by the sheet from the table and most of the uneven conditions caused at this point of the sheet forming operation.

65 Should the sheet break, it will still be car-

ried on by the movement of the table. When the table is driven in the manner above described, the leer rolls 28 will be driven at substantially the same speed as the travel of the sheet so as to draw the sheet over said table. The difference in the speed of travel between the flattening table and sheet may of course vary in different types of forming apparatus. However, for example, it is preferred that the travel of the table be approximately 20% less than the travel of the sheet but this is simply by way of illustration since the table may travel 30%, 40% or 50% slower than the sheet as conditions may seem to warrant. 70

To protect the rolls 11 and 12 and the sheet formed thereby from heat, gases, etc., it is preferred that lip tiles be used. At the closed end of the pot 5 is provided a relatively flat lip tile 29 while a second lip tile 30 is suspended above the molten glass in 85 advance of roll 12. A water cooled shield 31 may also be positioned between the roll 12 and the adjacent lip tile 30.

It is to be understood that the form of the invention herewith shown and described is 90 to be taken as the preferred embodiment of the same, and that various changes in the shape, size and arrangement of parts may be resorted to without departing from the spirit of the invention or the scope of the sub- 95 joined claims.

I claim:—

1. In the manufacture of sheet or plate glass, that step consisting in supporting a moving sheet of glass while in a semi-plastic condition upon a moving surface traveling in the same direction but at a different speed so that there is sliding engagement between said sheet and supporting surface. 100

2. In the manufacture of sheet or plate glass, that step consisting in supporting a moving sheet of glass while in a semi-plastic condition upon a moving surface traveling in the same direction as said sheet but at a relatively slower speed so that the sheet is 110 dragged over the supporting surface in sliding engagement therewith.

3. In the manufacture of sheet or plate glass, those steps consisting in advancing the sheet in a generally horizontal direction 115 while in a semi-plastic condition, and in supporting the sheet upon a moving surface traveling in the same direction but at a different speed, so that there is sliding engagement between said sheet and supporting surface. 120

4. In the manufacture of sheet or plate glass, those steps consisting in advancing the sheet in a generally horizontal direction while in a semi-plastic condition, and in supporting the sheet upon a moving surface 125 traveling in the same direction but at a relatively slower speed so that the sheet is dragged over the supporting surface in sliding engagement therewith.

5. In the manufacture of sheet or plate 130

glass, those steps consisting in supporting a moving sheet of glass while in a semi-plastic condition upon a movable supporting surface, causing said surface to move in the same direction as the sheet, and in advancing the sheet at a different speed than the supporting surface so that there is sliding engagement between the two.

5 6. In the manufacture of sheet or plate glass, those steps consisting in forming the sheet at a predetermined speed, carrying it forwardly in a generally horizontal direction at the same speed, supporting said sheet while still in a semi-plastic condition upon a horizontal supporting table, and in causing said table to move in the same direction as the sheet but at a different speed so that there is sliding engagement therebetween.

10 7. In the manufacture of sheet or plate glass, those steps consisting in supporting a moving sheet of glass while in a semi-plastic condition upon a movable supporting surface, causing said surface to move in the same direction as the sheet, and in advancing the sheet at a relatively faster speed than the supporting surface so that said sheet is dragged over said surface in sliding engagement therewith.

15 8. In the manufacture of sheet or plate glass, those steps consisting in forming a sheet of glass at a predetermined speed, carrying it forwardly in a generally horizontal direction at the same speed, supporting the sheet while still in a semi-plastic condition upon a horizontal supporting table, and in causing said table to move in the same direction as the sheet but at a relatively slower speed so that the sheet is dragged over said surface in sliding engagement therewith.

20 40 Signed at Lancaster, in the county of Fairfield and State of Ohio, this 19th day of June, 1929.

WILLIAM WILDERMUTH.

45

50

55

60

65